

P. AZARIA.

METHOD FOR OBTAINING METALLIC ATTACHMENTS FOR INCANDESCENT LAMPS.  
APPLICATION FILED JULY 28, 1909.

946,192.

Patented Jan. 11, 1910.

2 SHEETS—SHEET 1.

Fig. 1



Witnesses:  
N. Strohmeier  
R. G. Bent

Inventor:  
Pierre Azaria  
Kenny Goldsmith, M. D.  
Attala

P. AZARIA.

METHOD FOR OBTAINING METALLIC ATTACHMENTS FOR INCANDESCENT LAMPS.  
APPLICATION FILED JULY 28, 1909.

946,192.

Patented Jan. 11, 1910.

2 SHEETS—SHEET 2.

Fig.2.



Witnesses:  
D. Rockwood  
J. C. Smith.

Inventor:  
Pierre Azaria,  
of New York,  
N. Y.,  
Oct. 5, 1910.

# UNITED STATES PATENT OFFICE.

PIERRE AZARIA, OF PARIS, FRANCE.

## METHOD FOR OBTAINING METALLIC ATTACHMENTS FOR INCANDESCENT LAMPS.

946,192.

Specification of Letters Patent. Patented Jan. 11, 1910.

Application filed July 28, 1909. Serial No. 510,100.

To all whom it may concern:

Be it known that I, PIERRE AZARIA, citizen of the French Republic, residing at Paris, Department of the Seine, in France, have 5 invented certain new and useful Improvements in Methods of Obtaining Metallic Attachments for Incandescent Lamps; and I do hereby declare the following to be a full, clear, and exact description of the invention, 10 such as will enable others skilled in the art to which it appertains to make and use the same.

The lighting filaments of incandescent lamps are generally fixed to their metallic 15 holders by means of a paste having carbon or ground metal for a base and containing a plastic material which becomes hard under the action of heat. The attachment thus obtained is sufficiently steady and a rather 20 good electric conductor but has the great inconvenience of retaining in its pores occluded gases which are very difficult to eliminate during the vacuum operation.

If in incandescent lamps metallic filaments are used, it is possible to connect these filaments to their holders by means of a connection formed entirely with molten metal.

This invention consists in a new method of 30 autogenous soldering using only the radiant heat of accessory incandescent bodies and allowing of obtaining a very strong and non-porous joint. To carry out this peculiar method of soldering the metallic holders, generally, consisting of wires of nickel of an alloy 35 of nickel fixed in star fashion on a glass tube are terminated at the end where the soldering has to be effected by a very small eye or loop allowing of guiding the filament. The 40 latter is suspended from hooks or rings of metal, carbon, or other material, fixed in star fashion on a glass tube placed in the axis of the lamp. Sometimes the hooks or rings serve only to maintain the filament during 45 the soldering operation and are afterward removed. The glass tube which carries the filaments is placed in a closed space in which gases can be caused to circulate. Near each holder, at a distance of less than a millimeter 50 and below the point to be soldered, an electric conductor is placed which is capable of being quickly brought to a very high temperature by the passage of an electric current. The conductors may be formed of rods, wires, strips or the like, of a refractory material such for example as platinum or

carbon. There may be a special conductor corresponding with each part to be soldered or a single conductor of a special shape may be employed passing near all the points 60 where a soldering has to be effective. All being thus prepared, a reducing gas, which is a good conductor of heat, such as hydrogen is introduced into the said space and an intense electric current is caused to pass 65 through the conductor or conductors. Being instantaneously brought to a white red heat the conductor or conductors, by radiation and by virtue of the calorific conductivity of the gas heat the ends of the metallic 70 holders placed very near and above. The metal of these supports melts and forms, by capillary attraction, a very small metallic sphere which firmly incloses the branch of the filament in its center, thus forming a 75 perfect autogenous soldering from a mechanical and electric point of view, between the filament and its metallic holder. In a moment all the soldering of the lamp comprising several filaments can be effected in this 80 manner. The execution of these solderings is, in a way, automatic. As soon as the small sphere of melted metal inclosing the branch of the filament has been formed at the end of a support the distance to the incandescent 85 conductor increases sufficiently to stop the fusion without it being necessary to extinguish the heating conductor.

The accompanying drawing gives by way of example an apparatus which allows the 90 execution of this process.

Figure 1 is an elevation view of this apparatus. Fig. 2 is a plan view.

This apparatus comprises a glass bell 1 located on a plate 2 covered by a sheet of 95 india rubber 3. A pipe 4 allows to exhaust the air from the bell or to introduce a gas in the same, and serves also as supports for the central stem 6 of the lamp in fabrication. The lighting body is constituted by 100 filaments 7 suspended to insulated hooks 8. The filaments are electrically connected by the intermediary of V-shaped rods 9. These rods are fixed with the filaments by means of the process object of the invention. Two 105 uprights 10, 10 are located on a plate 11 and insulated from the same. Each of them bears pincers 12 and 13. The pincers 12 are electrically connected to the upright and the pincers 13 are insulated from the 110 same by a blade of mica 5. Between the pincers 12 and 13 is located a thin conductor

14 of refractory material which passes near the points to be welded. The pincers 13 13 are connected by a wire 15. When everything is in place for operation, vacuum is 5 made in the bell, and hydrogen is introduced. An electrical current adduced to the apparatus by the upright passes in the conductor 14 and the radiant heat produces the melting of the extremities of the V-shaped 10 rods 9, forming thus strong joints.

The use of this soldering process is not limited to the manufacture of incandescent lamps, but may also be employed when two metallic wires are to be soldered in order 15 to obtain strong joint and conductor.

I claim:

1. A process of autogenous soldering for connecting the metallic filaments of incandescent lamps to their holders, consisting 20 in causing an intense electric current to

pass through conductors of refractory material placed near the points where the soldering is to be effected and heating them by radiation.

2. A process of autogenous soldering for 25 connecting the metallic filaments of incandescent lamps to their holders, consisting in causing an intense electric current to pass through conductors of refractory material placed near the points where the soldering 30 is to be effected and heating them by radiation, the operation taking place in an atmosphere of hydrogen or any other reducing gas which is a good conductor of heat.

In testimony whereof I affix my signature, 35 in presence of two witnesses.

PIERRE AZARIA.

Witnesses:

H. C. COXE,  
GEORGES BOUJU.